

## UNITED STATES PATENT OFFICE

2,507,110

## COLOR FORMING PHOTOGRAPHIC DEVELOPMENT UTILIZING AMINO-N-HYDRO-CARBON SUBSTITUTED BETA-AMINO-ACRYLAMIDE COUPLERS

Robert Mitchell Leekley, Chicago, Ill., assignor to  
E. I. du Pont de Nemours & Company, Wil-  
mington, Del., a corporation of DelawareNo Drawing. Application July 11, 1946,  
Serial No. 682,933

15 Claims. (Cl. 95—6)

1

This invention relates to processes of color photography and to compositions and elements therefor which utilize substituted beta-aminoacrylamides as dye intermediates or color formers. It also relates to certain substituted beta-aminoacrylamides as new compounds and to their preparation.

An object of this invention is to provide improvements in the art of color photography. A related object is to provide new color-yielding elements, compositions, and processes. A further object is to provide photographic elements with color-yielding layers which do not have a deleterious effect on silver halide grains. A still further object is to provide a new class of color formers for the color-coupling development of silver halide images. Still other objects will be apparent from the following description of the invention.

It has been discovered that amino-N-substituted beta-aminoacrylamides may advantageously be employed in the color-coupling development of exposed silver halide images. They can be used in colloid layers of photographic elements or in alkaline developer solutions. The types which are fast to diffusion in water-permeable colloid layers can be advantageously used in colloid-silver halide emulsion layers or in coactive color-yielding colloid layers adjacent to colloid-silver halide emulsion layers or they may be dissolved in or dispersed in developer solutions with the aid of hydrotropic or dispersing agents. The mobile types are suitable for use in alkaline developer solutions according to well-known principles. They may be incorporated in the developer by any convenient method, such as by stirring in a solution of the color former in a water-miscible organic solvent.

The N-substituted beta-aminoacrylamides can readily be made by reacting a primary or secondary amine with a beta-ketoamide color former, that is, a beta-ketoamide which is capable of reacting with an oxidized primary aromatic amino developing agent to form an azomethine dye. A large number of such beta-ketoamide compounds are known. Suitable ones are described in United States Patents 2,108,602, 2,283,276, 2,299,641, and 2,319,426. They are reacted with the amine (preferably in excess) in a solvent or diluent for the beta-ketoamide. In the case of the normally gaseous amines or those which have a high vapor pressure they are reacted under pressure in a closed reaction vessel. When primary amines are used, the remaining hydrogen atom on the nitrogen atom of the beta-amino

2

group may be acylated by treatment with an acyl halide or carboxylic acid anhydride.

A class of substituted beta-aminoacrylamides useful in the compositions and processes described above may be prepared from beta-keto-amides of the formula



10 where



is an acyl radical of an aliphatic, aromatic, or heterocyclic acid  $RCOOH$  and Ar is an aromatic hydrocarbon nucleus. The products so prepared may be represented by the formula



where R' is a hydrocarbon radical; R'' is hydrogen, an acyl radical, or an aliphatic hydrocarbon radical; R has the same significance as in Formula 1; and Ar is an aromatic hydrocarbon nucleus. Thus, Ar may be a benzene, naphthalene, or diphenyl nucleus, unsubstituted or substituted by various groups common in color formers, e. g., nitro, carboxy, alkyl, aryl, cycloalkyl, alkoxy, halogen, etc.

When acylacetamides of aromatic aminoaldehydes or their lower acetals are used for reaction with the amines there is produced a new class of compounds which have considerable utility as color formers and also as intermediates for the preparation of high molecular weight color formers. Thus, they may be reacted with hydroxyl polymers, e. g., polyvinyl alcohol, partially hydrolyzed hydrophilic polyvinyl esters, hydrolyzed and partially hydrolyzed hydrophilic ethylene/vinyl acetate interpolymers (described in United States Patent 2,386,347), etc., to form hydroxyl polymer acetal color formers. Thus the acylacetamides of meta-aminobenzaldehyde and its acetals with monoalkanols of 1 to 4 carbon atoms and 1,2- and 1,3-alkanediols of 2 to 4 carbon atoms are suitable reactants. They may be prepared by acylation of an acetal of the amino-benzaldehyde with an acyl acetic acid methyl or ethyl ester, followed, if desired, by hydrolysis to the free aldehyde.

The N-substituted beta-aminoacrylamidobenzaldehyde and their lower acetals have the advantage in the preparation of acetals with hydroxyl polymers that no interaction between the alde-

3

hyde group and an active methylene group takes place as may occur in the case of the unsubstituted compounds. In addition, complex reactions which may lead to cross linking of the hydroxyl polymer molecules are avoided.

The invention will be further illustrated by the following examples. All parts are by weight.

### Example 1

Into a cooled mixture of 25 parts acetoacetanilide in 277 parts of benzene is condensed 75 parts of dimethylamine. The reaction vessel is sealed and the mixture allowed to stand at 25°-30° C. under the pressure developed for 18 hours. The reactor is cooled to about 5° C. before opening. An additional 285 parts benzene is added and the excess dimethylamine, water, and about half of the benzene are removed by distillation. The residue is cooled to room temperature and filtered to yield 24 parts of white crystalline beta-dimethylaminocrotonanilide melting at 165°-166.5° C. (Knorr, Ber. 25, 777 reports 160° C.). The product has the structural formula



A latent silver photographic image is developed by treatment of the emulsion for five minutes with a developing solution by adding a solution of two parts beta-dimethylaminocrotonanilide in 63 parts of 95% alcohol to 1,000 parts of the stock solution prepared from the following ingredients by dissolving in 500 parts of water and diluting to 1,000 parts:

|                                        | Parts |
|----------------------------------------|-------|
| para-Aminodiethylaniline hydrochloride | 2     |
| Sodium sulfite (anhydrous)             | 2     |
| Sodium carbonate (anhydrous)           | 20    |
| Water to make                          | 1000  |

After washing with water, bleaching the silver image with 4% potassium ferricyanide solution, and fixing with 25% sodium thiosulfate solution, a sharp, bright-yellow image remained.

### *Example II*

Reaction of 25 parts acetoacetanilide with 30 parts of methylamine in 227 parts of benzene under the conditions of Example I, yielded 23 parts of beta-methylaminocrotonanilide melting at 140°-141° C. (Knorr, Ber. 25, 771 reports 144.5° C.). The product has the formula



Use of this color former for development of a silver image as described in Example I, yielded a yellow image.

*Example III*

Reaction of 75 parts of m-acetoacetamido-benzaldehyde ethylene glycol acetal (prepared by Procedure A below) with 80 parts dimethylamine in 340 parts of benzene, after the manner of Example I, yields 85 parts of m-(beta-dimethylaminocrotonamido)benzaldehyde ethylene glycol acetal of the formula



After recrystallizing from benzene this compound

4

melts at 164°-165° C. Analysis, calculated for  $C_{15}H_{20}N_2O_3$ : C=65.21; H=7.25. Found: C=65.28, 65.14; H=7.25, 7.15.

Five parts of this compound are added to 100 parts of a gelatin emulsion and the mixture is coated on paper, exposed, developed, fixed, bleached, and fixed as described in Example I to give a bright-yellow image free of fog.

*Example IV*

10 A mixture containing 20 parts of finely di-  
15 vided polyvinyl alcohol (completely hydrolyzed  
and having a 4% aqueous solution viscosity of  
18 to 24 centipoises at 20° C.), 5 parts m-(beta-  
15 dimethylaminocrotonamido)benzaldehyde ethyl-  
16 ene glycol acetal (see Example III) and 100 parts  
17 of glacial acetic acid, is heated at 60° C. for three  
18 hours and then cooled. The suspended product  
19 is removed by filtering, and is washed by repeated  
20 slurring with methanol. A solution is prepared  
21 by stirring together at 50°-60° C. ten parts of  
22 this polymer, 40 parts of 95% ethyl alcohol, 150  
23 parts of water, and sufficient sodium hydroxide  
24 to bring the pH to about 8. To one-half of this  
25 solution is added 31 parts of 3N ammonium  
26 bromide and two parts of 0.5N potassium iodide.  
27 The mixture is stirred at 40° C. while adding a  
28 solution of 29 parts of 3N silver nitrate, 50 parts  
29 of water, and 17 parts of 28% ammonium hy-  
30 droxide during one minute. After stirring for  
31 a total of one-half hour, 150 parts of 15% sodium  
32 sulfate solution is added. The precipitated silver  
33 halide/color-former emulsion is washed for one  
34 hour in running water, after which the excess  
35 water is drained off. The remainder of the orig-  
36 inal polymer solution is added and the mixture  
37 stirred at 65° C. for one-half hour. After cool-  
38 ing to 25° C., the emulsion is coated on baryta-  
39 sized white paper. The resulting paper is ex-  
40 posed to form a latent image, then developed in  
a solution of the following composition prepared  
by dissolving the ingredients in 500 parts of water  
and diluting to 1,000 parts.

|                                        | Parts |
|----------------------------------------|-------|
| 45 p-Aminodiethylaniline hydrochloride | 2     |
| Potassium sulfite (anhydrous)          | 2     |
| Sodium carbonate (anhydrous)           | 20    |
| Potassium bromide                      | 1     |
| Water to make                          | 1000  |

50 The paper is then washed, bleached in 4% potassium ferricyanide, fixed in 25% sodium thiosulfate, and washed. The resulting yellow image is sharp and free of fog.

*Example V*

55 Reaction of 75 parts of m-acetoacetamido-benzaldehyde ethylene glycol acetal with 80 parts methylamine in 680 parts of benzene by the method described in Example I yields 70 parts  
 60 of m-(beta-methylaminocrotonamido)benzaldehyde ethylene glycol acetal melting at 75°-77° C. and having a formula similar to that of Example III but containing 1 methyl group attached to the beta-amino nitrogen atom. Analysis, calculated for  $C_{14}H_{18}N_2O_3$ : C=64.12; H=6.87; and N=9.36. Found: C=65.23, 65.15; H=7.30, 7.31; and N=10.05, 10.19. When added to a developer solution as in Example I, the product gives a clear yellow image.

70

*Example VI*

A solution of 26.2 parts of the m-(beta-methyl-aminocrotonamido)benzaldehyde ethylene glycol acetal and 15 parts of pyridine in 138 parts methylene chloride is cooled in an ice bath to 5° C.

and a solution of 14 parts of benzoyl chloride in 35 parts of methylene chloride is added with stirring. After five minutes the mixture is removed from the ice bath and allowed to warm up to room temperature while stirring is continued. The product is precipitated by addition of petroleum ether and recrystallized from acetone to give m-[beta-(N-methyl-benzamido)-crotonamido]benzaldehyde ethylene glycol acetal melting at 147°-148° C. and having the formula 10



When incorporated in a gelatin emulsion and processed as in Example III, the product gives 20 a bright yellow image free of fog.

*Example VII*

To a suspension of 30 parts of polyvinyl alcohol (see Example IV) in 75 parts of dioxane, is added 25 7.5 parts of m-[beta-(N-methylbenzamido)crotonamido]benzaldehyde ethylene glycol acetal and 0.1 part of 85% phosphoric acid. The mixture is heated with stirring for eight hours at 70° C. The product is filtered off, washed repeatedly with methanol, and dried.

A solution is prepared by stirring ten parts of this polymer with 40 parts of 95% ethyl alcohol, 150 parts of water, and 0.5 part of sodium hydroxide. An emulsion prepared as described in Example IV coats smoothly on baryta-sized white paper and, when exposed and developed, yields a yellow photographic image.

*Example VIII*

A solution of 31.1 parts of m-benzoylacetamidobenzaldehyde ethylene glycol acetal in 180 parts of benzene is cooled and dimethylamine is passed in until a weight gain of 30 parts is noted. Two layers separate. The reaction vessel is sealed and shaken for 24 hours, then allowed to stand at room temperature for three days, by which time the layers coalesce. It is then cooled and opened and the excess dimethylamine, water, and benzene are removed by distillation, the last part under reduced pressure. The residual oil, 33 parts, is m-(beta-dimethylamino-cinnamido)benzaldehyde ethylene glycol acetal having the following probable structure:



When exposed photographic paper is developed in a color developer containing this color former as in Example I, a clear, bright yellow image having excellent spectral characteristics is obtained.

*Example IX*

To a solution of 10.3 parts of m-(beta-dimethylamino-cinnamido)benzaldehyde ethylene glycol acetal, 160 parts of ethanol, 2.25 parts of o-sulfo-benzaldehyde, 45 parts of water, and three parts of 85% phosphoric acid is added 45 parts of polyvinyl alcohol and the suspension is stirred for one hour at 80° C. The polymer is collected on a filter, washed thoroughly with methanol and acetone, and dried.

A solution is prepared by stirring ten parts of this polymer with 20 parts of ethanol and 170 parts of water at 80° C. for 15 minutes. The resulting clear solution is used to prepare an emulsion as described in Example IV, which is coated on paper and processed to an exceptionally bright-yellow image.

*Procedure A*

A mixture of 425 parts of ethyl acetoacetate, 1.5 parts of dry pyridine and 525 parts of dry xylene is heated to the boiling point and a mixture of 445 parts of m-aminobenzaldehyde ethylene glycol acetal, three parts of dry pyridine and 525 parts of xylene is added with stirring over a period of three hours. The ethanol formed is allowed to distill as fast as it is produced. Heating is continued for one hour after addition is complete by which time distillation of ethanol ceases. The reaction mixture is allowed to cool to room temperature and the white crystalline solid is collected on a filter. The cake is slurried in 2600 parts of 5% sodium hydroxide and filtered. The filtrate is saturated with carbon dioxide and the solid is collected on a filter, washed with water, and dried. The yield is 368 parts (58%) of white crystalline solid, melting at 85°-86° C. having the structural formula



Analysis: Calculated for  $C_{13}H_{15}NO_4$ : C=62.7; H=6.0; N=5.6. Found: C=62.8; H=6.5; N=5.6.

The acetal can be hydrolyzed by dissolving it in acetone and adding a small amount of 1N phosphoric acid. Upon cooling the m-acetocetamidobenzaldehyde crystallizes out and can be recrystallized from acetone and has a melting point of 96.5° to 97.5° C.

Analysis: Calculated for  $C_{11}H_{11}NO_3$ : C=64.4; H=5.4; N=6.8. Found: C=64.4; H=5.5; N=6.8.

In place of the specific amines described in the above examples, there may be substituted various other primary and secondary amines including propylamine, dipropylamine, butylamine, di-butylamine, cyclohexylamine, dicyclohexylamine, 50 benzylamine, dibenzylamine, betanaphthylamine, aniline, p-chloroaniline, piperidine, ethanolamine, and diethanolamine. When a long chain amine, e. g., dodecylamine, is used the dye intermediate is rendered non-diffusing and 55 is useful in the preparation of multilayer color films.

Similarly in place of the specific acylacetamides as set forth in the above examples there may be substituted other such compounds including N-phenylacetanilide, other aryl-acetanilides including benzoylacetanilides, N-methyl benzoylacetanilide and furoylacetanilides as well as the beta-ketoamides disclosed in the patents listed above. When the beta-ketoamides contain two acylacetamide radicals, substituents may be introduced on one or both of the keto groups.

The reaction is carried out under suitable conditions according to the reactivity of both the beta-ketoamides and the amine. When the amine is a low molecular weight aliphatic amine, the reaction is carried out at room temperature under the pressure developed by the amine in a closed vessel. Higher pressures can be developed by heating. When higher molecular

weight amines are used, the reaction may be carried out at atmospheric pressure or at elevated temperatures, if necessary, by refluxing in a solvent. The time of reaction varies depending on the reactants and can be from 1 to 100 hours.

Various other solvents or diluents may be used, for example, carbon tetrachloride, chloroform, toluene, xylene, or dioxane.

Acylating agents which can be used to acylate the reaction products prepared from primary amines include, in addition to benzoyl chloride utilized in Example V, acetyl chloride, acetic anhydride, benzenesulfonyl chloride, toluenesulfonyl chloride, and ethyl chlorocarbonate. In addition, it is possible to prepare the N-acyl-amino derivatives of the color-formers by direct reaction of the color former with the appropriate amide. An example of this type is the reaction of acetamide with acetoacetic ester (Canzoneri and Spica, "Gazzetta Chimica Italiana" 14, 491).

The color formers may be incorporated into emulsions conventionally by dissolving them in a solvent which does not affect the sensitivity of the emulsion and intimately mixing the same with the water-permeable colloid binder, e. g., a gelatin solution or emulsion. A small amount of an alkali metal base is sometimes advantageous in obtaining a rapid and uniform dispersion of the color former throughout the emulsion. The compounds are, remarkably free of deleterious effects on the photographic sensitivity and chromatic response characteristics of silver halide emulsions, e. g., silver chloride, silver bromide, and silver chlorobromide, silver-bromide-iodide, etc. emulsions. They may likewise be used in conjunction with the known sensitizing dyes which render the emulsions sensitive to certain additional wave length regions of light. They may also be used in conjunction with emulsion desensitizers, surface modifiers, and emulsion hardening agents and binding agents other than gelatin, e. g., agar agar, hydrophilic cellulose derivatives, e. g., ethyl cellulose, hydrolyzed cellulose acetate, hydrophilic polymers, e. g., polyamides and hydrolyzed ethylene/vinyl acetate interpolymers of United States Patent No. 2,397,866.

They may be incorporated in developer solutions in various known manners, for example, by dissolving them in an organic solvent miscible with water and adding the solution to the aqueous developer solution. They may, if their solubility is sufficient, be added directly to the bath. In some cases, the use of dispersing agents, such as alkylated naphthalene sulfonates, higher aliphatic alcohol sulfates, higher alkyl sulfonates, mineral oil sulfonates, Turkey red oil, etc., may be employed.

Other developer solutions with which the novel color formers may be used as described in United States Patent 2,299,641.

An advantage of the invention resides in the fact that it provides a large class of utilizable color formers. Another advantage is that the color formers may be obtained from available initial materials.

The real advantage appears when complex molecules containing several functional groups are used. An example of this is *m*-acetoacetamidobenzaldehyde ethylene glycol acetal. When this product is used to prepare polyvinyl acetals by acetal interchange with polyvinyl alcohol in such solvents as dioxane or acetone, side reactions often occur which lead to partial insolubility.

bilization of the polyvinyl alcohol. These side reactions are prevented by protection of the active methylene group of the acetoacetanilide through conversion to the substituted beta-aminoacrylamidobenzaldehyde. These compounds can then be used to make soluble polyvinyl acetal color formers. The substituted beta-aminoacrylamido derivatives of acylacetamides of m-aminobenzaldehyde acetals are new compounds.

As many widely different embodiments of this invention can be made without departing from the spirit and scope thereof, it is to be understood that the invention is not to be limited except as defined by the claims.

What is claimed is:

1. A photographic developer composition comprising a primary aromatic amino developing agent and an aminonitrogen-hydrocarbon-substituted beta-aminoacrylamide.
  2. A photographic developer solution containing a primary aromatic amino developing agent and an aminonitrogen-hydrocarbon-substituted beta-aminoacrylamide.
  3. A photographic developer solution containing a primary aromatic amino developing agent, an alkali, and an aminonitrogen-mono-aryl-substituted beta-aminocrotonamide.
  4. A photographic developer solution containing a primary aromatic amino developing agent and a compound of the formula



35 wherein R' is a hydrocarbon radical, R'' is a member taken from the group consisting of hydrogen, acyl, and hydrocarbon radicals, and Ar is an aromatic hydrocarbon nucleus.

5. A photographic element comprising a support bearing light-sensitive silver halides and at least one water-permeable colloid layer containing an aminonitrogen-hydrocarbon-substituted beta-aminoacrylamide.

6. A photographic element comprising a support bearing light-sensitive silver halides and at least one water-permeable colloid layer containing an N-mono-hydrocarbon substituted beta-aminoacrylamide.

7. A photographic element comprising a support bearing light-sensitive silver halides and at least one water-permeable colloid layer containing a compound of the formula



wherein R' is a hydrocarbon radical, R'' is a member taken from the group consisting of hydrogen, acyl, and hydrocarbon radicals, and Ar is an aromatic hydrocarbon nucleus.

60 8. The process which comprises developing a photographic element containing an exposed silver halide layer with a primary aromatic amino developing agent in the presence of an amino-nitrogen-hydrocarbon-substituted beta - amino-acrylamide.

9. A photographic developer solution containing a primary aromatic amino developing agent and a compound of the formula



wherein R' is a hydrocarbon radical, R'' is a member taken from the group consisting of hydrogen, acyl, and hydrocarbon radicals, and Ar is an aromatic hydrocarbon nucleus.

10. A photographic element comprising a support bearing light-sensitive silver halides and at least one water-permeable colloid layer containing a compound of the formula



wherein R' is a hydrocarbon radical, R'' is a member taken from the group consisting of hydrogen, acyl, and hydrocarbon radicals, and Ar is an aromatic hydrocarbon nucleus.

11. The process which comprises developing a photographic element having an exposed silver halide layer with a developer solution containing a primary aromatic amino developing agent and an alkali in the presence of a beta-methylaminocrotonanilide.

12. The process which comprises developing a photographic element having an exposed silver halide layer with a developer solution containing a primary aromatic amino developing agent and an alkali in the presence of a beta-dimethylaminocrotonanilide.

13. A photographic element comprising a support bearing a colloid silver halide emulsion layer containing a m-(beta-dimethylaminocrotonamido)benzaldehyde ethylene glycol acetal.

14. A photographic developer solution containing a primary aromatic amino developing agent and a compound of the formula:



wherein R is a radical taken from the group

consisting of aliphatic and aromatic hydrocarbon radicals, R' is a hydrocarbon radical, R'' is a member taken from the group consisting of hydrogen, acyl, and hydrocarbon radicals and Ar is an aromatic hydrocarbon nucleus.

15. A photographic element comprising a support bearing light-sensitive silver halides and at least one water-permeable colloid layer containing a compound of the formula:



wherein R is a radical taken from the group consisting of aliphatic and aromatic hydrocarbon radicals, R' is a hydrocarbon radical, R'' is a member taken from the group consisting of hydrogen, acyl, and hydrocarbon radicals and Ar is an aromatic hydrocarbon nucleus.

ROBERT MITCHELL LEEKLEY.

#### REFERENCES CITED

The following references are of record in the file of this patent:

#### UNITED STATES PATENTS

| Number    | Name        | Date           |
|-----------|-------------|----------------|
| 2,282,001 | Russell     | May 5, 1942    |
| 2,307,399 | Frohlich    | Jan. 5, 1943   |
| 2,319,426 | Middleton   | May 18, 1943   |
| 2,325,331 | Martin      | July 27, 1943  |
| 2,359,274 | Wilson      | Sept. 26, 1944 |
| 2,407,207 | Salminen    | Sept. 3, 1946  |
| 2,407,210 | Weissberger | Sept. 3, 1946  |